

## UNITED STATES PATENT OFFICE

1,968,418

## MANUFACTURE OF FIBER PRODUCTS

Treadway B. Munroe and Marion D. Coulter,  
Chicago, Ill.No Drawing. Application October 30, 1930,  
Serial No. 492,359

7 Claims. (Cl. 92—21)

In the manufacture of paper, fiber board, molded fiber products, fiber insulation board, various types of felts such as roofing felt, and in the manufacture of many more or less similar products it is common to incorporate thereinto, in the process of manufacture, various water-proofing, fire-proofing, insect-repellent, insect toxic, fungicidal, and like substances hereinafter referred to as proofing agents. This invention is directed to 10 the method of incorporating the above-mentioned substances into the fiber product during its process of manufacture.

The particular object of this invention is to provide a new manner of procedure in the manufacture of products such as above named, whereby such treatment as is desired may be applied more readily, more economically, and more uniformly than is accomplished by present practices.

20 As an example of the application of the principles of this invention, the process will be particularly described in connection with a treatment employed to render fiber insulation board insect, and fungi-proof. A well known fiber insulation board is manufactured with a major percentage of bagasse fiber and a minor percentage of wood fiber pulp, which latter portion may conveniently be added as pulped newspaper.

The board is formed from a water suspension 30 of the fiber content of close to 0.75%. According to present practice, processes for the inclusion of treatments to incorporate materials such as insecticides and fungicides have comprehended the addition of the necessary chemicals or 35 materials at a point at which the stock is termed "half stock", that is, at a point where all the fiber is in suspension, but where it has not been given the final dilution, and at which point the consistency is ordinarily about 1½ to 2%, or even slightly higher. As distinguished from past practice, it has been found that by adding the fungicide and insecticide to the pulped news print prior to the addition thereof to the primary fiber, various important advantages are obtained.

45 Some of the advantages of this improved process of treatment are in that the pulped news print is used in a quantity approximately only one-third that of the primary fiber. The fiber derived from the news print is more readily hydrated than the primary fiber and, as hydrated fiber, it exposes a large surface whereby adsorption is increased. Other advantages are that news print is pulped and handled at relatively high consistency—that is, at about 4 to 5%—and therefore, due to the smaller amount and the

higher consistency, the desired treatment may be more uniformly applied. With the treatment applied initially to a minor portion of the stock, losses are smaller in that a closed system may be maintained, or even if a closed system is not used, losses are much reduced due to the fact that the quantity of water in this stock is much less than the quantity of water present after the major and minor portions of fiber have been mixed and diluted to half stock.

In treating an insulating board comprising, roughly, 75% bagasse and 25% pulped news print, the procedure is as follows:

The pulped news print at a rather high consistency—about 4 to 5%—has added thereto an appropriate amount of ferric chloride and arsenious acid, say about 3½%, based on the dry weight of the fiber, with a ratio of As : Fe of about 1¼ : 1. The pH is then adjusted to the appropriate point between pH 4.0 and pH 12.0, dependent upon the presence of electrolytes, etc., to cause a change of the ferric chloride to hydrous ferric oxide which is adsorbed by the fiber and which in turn adsorbs the arsenic, whereby the arsenic is adhered to the fiber.

The pulped news print with its adhered arsenic is then thoroughly mixed with the bagasse fiber in proportions of about one to three, diluted to proper consistency for board formation, and then formed into the desired board on an appropriate board-forming machine.

The general scheme of this invention is applicable in any use wherein it is possible to apply it to a portion of the total fiber used, and particularly where it can be applied to the finer and more highly hydrated fiber of the furnish.

The principles are applicable in any case wherein the treatment is accomplished by adsorption by the fiber, or precipitation on the fiber. It may be employed in connection with waterproofing, since in products of the type involved the waterproofness is obtained by the aggregate of many particles lying on or between fibers rather than from films formed around individual fibers, and in fireproofing the protection is afforded by uniform distribution of the fireproofing materials rather than by what might be termed integral distribution, considered as mass treatment of all the elements, but which due to difficulties of treatment may not comprise uniform treatment.

Whereas the treatment has been described for one particular application, the principles are applicable in sizing, for example, with rosin and alum, wax, etc., and in fireproofing with ferrous

oxalate formed as by interaction of ferrous sulphate and oxalic acid, or in fact, the process is applicable for any treatment of the general type of those particularly mentioned. In the claims 5 the word "proofing" is employed particularly to designate treatment of the fiber with an insect and fungi toxic substance.

It is obvious that those skilled in the art may vary the details of construction as well as the 10 steps constituting the method without departing from the spirit of the invention, and therefore it is not desired to be limited to the foregoing except as may be required by the claims.

What is claimed is:—

15 1. The method of proofing a fibrous product which consists in adding to a fraction thereof ferric chloride and arsenious acid, and then admixing said fraction with the remainder of the fibrous material to form said product.

20 2. A fiber product of the type described comprising a fiber portion carrying an adhered proofing agent and integrally incorporated throughout the primary fiber comprising the product, and wherein the adhered proofing agent is a complex 25 arsenical resulting from interaction of ferric chloride and arsenious acid in dilute solution.

25 3. A fiber product of the type described comprising a fiber portion carrying an adhered proofing agent and integrally incorporated through-

out the primary fiber comprising the product, and wherein the adhered proofing agent comprises arsenious acid as an element of a substantially cold water insoluble colloidal complex.

4. The method of proofing a fibrous product 80 which consists in adding to a fraction thereof an adherent arsenical and subsequently admixing said fraction with the remainder of the fibrous material to form said proofed product.

5. A fiber product of the type described, comprising a fiber portion carrying an adherent proofing agent and integrally incorporated throughout the primary fiber comprising the product and wherein the adherent proofing agent comprises arsenious acid as an element 90 thereof.

6. A fiber product having a primary fiber content and a secondary fiber content, the secondary fiber content carrying an insect and fungi toxic chemical and integrally distributed throughout the primary fiber content thereof.

7. A fiber product having a primary fiber content and a secondary fiber content, the secondary fiber content carrying a substantially water insoluble adhered insect and fungi toxic arsenical, 100 the secondary fiber content integrally distributed throughout the primary fiber content.

TREADWAY B. MUNROE.  
MARION D. COULTER.

105

33

36

110

40

115

45

120

50

125

55

130

60

135

66

140

69

145

74

150